

Aug. 16, 1932.

G. R. ALDEN

1,871,647

METHOD FOR MAKING COLORED CREPE PAPER WITH  
INSOLUBLE DYES AND RESULTING PRODUCT  
Original Filed Nov. 12, 1926



*Trevor J. Alden  
Gardner R. Alden  
D. J. Balloch, C. Schumacher, H. H. Morris  
Assignors*

Patented Aug. 16, 1932

1,871,647

# UNITED STATES PATENT OFFICE

GARDNER R. ALDEN, OF FRAMINGHAM, MASSACHUSETTS, ASSIGNOR TO DENNISON MANUFACTURING COMPANY, OF FRAMINGHAM, MASSACHUSETTS, A CORPORATION OF MASSACHUSETTS

## METHOD FOR MAKING COLORED CREPE PAPER WITH INSOLUBLE DYES AND RESULTING PRODUCT

Original application filed November 12, 1926, Serial No. 147,959. Divided and this application filed April 2, 1930. Serial No. 441,140.

This invention relates to a method for the manufacture of non-bleeding colored crepe paper and to the resulting product.

It has been proposed and described in a co-pending application of Galen H. Sayler (Serial No. 139,176 filed October 2, 1926) issued as Patent 1,732,540, dated October 22, 1929, to produce colored crepe paper by treating a sheet of suitable paper with a dye solution and with a fixing solution, successively or simultaneously, and then creping the thus dyed sheet as by passing it through the usual creping bath and over a creping roll. In this course of procedure there are certain limitations and disadvantages which may arise in the course of practical operations which it is desirable to overcome or avoid. For example, in such processes some fixing reagents, such as aluminum sulfate or the like, cause the precipitation of the adhesive (which it is often desirable to provide in the creping bath), thus destroying it for further use. Moreover, the adhesive and some fixing agents or dyes tend to accumulate upon the creping roll and interfere with the proper creping operation, forming streaks or lines in the paper, and thus finally necessitate a thorough cleaning of this part of the machine. This is especially likely to occur when the creping roll is heated. Again, certain reagents (such as tannic acid and inorganic salts) may react with and corrode the surface of the iron creping roll. This makes it necessary to remove and regrind the roll to obtain a true cylindrical surface, involving a prolonged and difficult operation requiring a considerable amount of time and special equipment. On the other hand, acid resistant alloys would be extremely expensive, even if it were possible to provide them in sufficiently large sizes.

Accordingly, it is an object of the present invention to provide an improved method for making colored crepe paper, whereby such disadvantages and difficulties, when they occur, may be avoided and to produce a satisfactory non-bleeding colored crepe paper. Other objects will appear from the disclosure and claims.

The method of the invention includes gen-

erally the treatment of a sheet of paper with the dye solution or the fixing agent or such other reagent materials as may not deleteriously affect the creping bath or creping operation, then creping the sheet, and subsequently applying to the creped sheet such active reagent materials as may be required and in such a manner as substantially to preserve the creped structure of the sheet.

For example, a sheet of paper may be first treated with a dye solution inert with respect to the creping bath and creping apparatus, then creped (with or without the use of adhesive) and the dyed and creped sheet then treated with the appropriate fixing or other reagents. In such cases the dye solution may serve also as a creping bath and, if desired, a suitable adhesive may be added thereto or a separate creping bath may be employed.

A further improvement in the method may be effected by dissolving the fixing reagent (especially when applied after the creping operation) in such a solvent or in such concentration that it does not seriously affect or reduce the crepe of the sheet. On the other hand, the paper may first be treated with the fixing reagent (where the fixing reagent may be added to or contacted with the creping bath without detriment) and the paper then creped, and the creped paper subsequently treated with an appropriate dye solution.

A specific and representative instance of the application of the invention will now be described as carried out by means of the apparatus illustrated in the accompanying drawing in which

The figure is a diagrammatic side elevation of the several pieces of apparatus required.

Referring to the drawing, numeral 1 indicates a roll of the paper to be treated, which is carried upon a roller 2 rotatably mounted at 3. The creping apparatus 4 includes a guide roller 5, a flooding bar 6, a rubber roller 7, which dips into the solution 8 contained in tank 9. Above roller 7 and in pressure contact therewith is provided a creping roll 10 rotatably mounted and having a doctor blade 11 in close contact with its peripheral surface at the desire off-take point of 100.

the roll. An air nozzle or blower 12 is also positioned adjacent to the roll between the points of contact with roller 7 and with the doctor blade 11.

5 The means for imparting the subsequent treatment to the creped sheet (whether dye solution or fixing reagent) comprises a flooding bar or roller 13, a pair of compression rollers, including a lower roller 14 (which 10 may have a felted or other resilient and/or irregular surface), dipping into the solution 15 in tank 16, and an upper roller 17 which may or may not apply a treating solution, as desired. This apparatus is followed by 15 suitable drying apparatus, if necessary, and a rewinder or other gathering apparatus, not shown.

Appropriate dye solutions for use in the 20 operation of the method may be prepared as follows:

|                |                                                                          |            |    |
|----------------|--------------------------------------------------------------------------|------------|----|
| 1. For red:    | Erie fast scarlet 4 BA (Color Index #326—Schultz #279)                   | 5 lbs.     | 50 |
|                | Water                                                                    | 60 gallons |    |
| 2. For orange: | Pheno orange O (Color Index #621—Schultz #11)                            | 5 lbs.     | 55 |
|                | Water                                                                    | 60 gallons |    |
| 3. For orange: | Auramine (concentrated) (Color Index #655—Schultz #493)                  | 32 ounces  | 60 |
|                | Rhodamine 6 GDN ex (Color Index #752—Schultz #571, a xanthine basic dye) | 14 ounces  |    |
|                | Water                                                                    | 60 gallons |    |
| 4. For green:  | Auramine (concentrated) (Color Index #655—Schultz #493)                  | 60 ounces  | 65 |
|                | Methylene blue (Color Index #922—Schultz #659)                           | 80 ounces  |    |
|                | Water                                                                    | 60 gallons |    |

35 The adhesive used for facilitating and improving the creping operation (if any) may be glue, dextrine or the like and may be dissolved in the dye or in the fixing reagent solution or, as noted above, employed independently.

40 An active fixing agent (as for the dye solution 1 and 2 above mentioned) may consist, for example, of an aqueous solution of aluminum sulfate. Owing to the wetting and de-creping effect of water, it is desirable, as 45 later explained, to use a concentrated solution whenever it is applied to paper which has been previously creped. To this end a concentrated solution of ammonium sulfate may be added thereto. Thus, a solution containing both—15 lbs. aluminum sulfate, 180 50 lbs. ammonium sulfate, 60 gals. of water—has been found well suited for the purpose. The two salts may, however, be contained in 55 separate solutions, the concentrated ammonium sulfate solution being applied in the form of a spray, for example, and the aluminum sulfate solution (preferably though not necessarily concentrated) by means of the roller 14 or other device. The presence of 60 the second salt may serve the additional function of fireproofing the sheet.

Preliminary to the operation of the apparatus, the sheet 1 is drawn from roller 2 and passed over guide roller 5, beneath flooding 65 bar 6 and over roller 7, between roller 7 and

creping roll 10, over the surface of the creping roll to the doctor blade 11, from which it is carried under flooding bar or roller 13 and between the felted rollers 14, 17, and thence to the drying and take-up mechanism. The sheet may be drawn through the apparatus, but since this tends to stretch and remove the crepe effect, it is preferable to positively drive the several rollers in unison with each other, in the directions indicated by the arrows.

With the apparatus thus arranged, the dye solution, for example, such as that indicated by the first formula above given, is run into the tank 9, together with the adhesive if such is to be used. As already pointed out the dye solution may be separately applied to the sheet first and the sheet then passed through a creping solution in tank 9, but unless intermediate drying is resorted to, the dye and glue should be mutually inert in this order of procedure. The fixing solution (given above) is then placed in tank 16, or the alum solution only, and means provided (not shown) for spraying the ammonium sulfate solution upon the top of the sheet or upon roller 17.

The sheet of paper is now passed by rotation of the several rollers under a pool of the dye solution, which is carried upon its upper surface in the depression formed by the flooding bar 6, and distributed throughout the width of the sheet by the transverse contact of the bar. As the sheet proceeds and comes into contact with the surface of roller 7 (which is wet with the dye solution) it is wet upon its under surface, and as the sheet continues to pass between roller 7 and creping roll 10 it is firmly compressed and squeezed. This not only completes the uniform distribution of the solution throughout the sheet, both laterally and transversely through the sheet, but effectively expresses the surplus of the dye solution which thereupon passes through the sheet and flows down upon its upper surface and maintains the pool of dye solution adjacent to the flooding bar. The sheet is also thereby brought into intimate contact with the creping roll to which it firmly adheres until it reaches the doctor blade 11 which skives the sheet from the surface of the roll. In this removal of the sheet from the creping roll, the paper is repeatedly folded back upon itself, forming a succession of wrinkles therein. The size of the folds thus produced depends partly upon the angle at which the doctor blade is set with respect to the surface of the creping roll and upon the shape of doctor blade and is also governed by the degree of adhesion of the sheet to the roll surface. In general, the more firmly the sheet adheres to the roll, the more numerous and closely packed the folds of the crepe may be made, and the finer the creping produced. It is also possible to provide and pre-

serve a high crepe ratio by this procedure which is especially desirable. By "crepe ratio" is meant the proportion which a given length of the sheet bears to the length of the creped sheet resulting therefrom.

The creped sheet may be removed at this point and dried, if desired, and the subsequent treatment independently conducted at a later time, or it may pass directly and continuously to such treatment. In either case, the creped sheet, already colored is next subjected to the fixing treatment. For example, the sheet of crepe paper is passed under a pool of the solution held by flooding bar 13 and thence between the rollers 14 and 17. The lower roller dips into the bath of reagent 15 is thoroughly wet thereby and carries the solution up and applies it to the under surface of the creped sheet as it comes into contact therewith and distributes it more uniformly thereover as the paper passes under compression between the rolls.

While the wetting of crepe paper stock with water or dilute aqueous solutions always reduces the crepe ratio to a considerable extent or almost entirely destroys the creped structure, it is found that with concentrated solutions of certain inorganic electrolytes (for example, salts such as ammonium sulfate, sodium nitrate, sodium chloride, sodium sulfate, which are substantially neutral with respect to paper, to prevent deterioration of the sheet) this effect is practically negligible. Again, organic solvents have little or no destructive effect upon crepe paper and some organic liquids, such as alcohol, may contain as much as 50% of water and still remain ineffective toward the creped structure of a paper sheet. Accordingly, in any specific instance it is practicable to impart an initial crepe ratio to the paper of such an order that even though a part may be lost by the subsequent treatments indicated, there will be left a sufficiently high degree of creping in the finished sheet to be entirely satisfactory for the desired purpose.

Accordingly, to this end, the amount of fixing reagent solution applied to the sheet is kept low and a relatively high concentration of neutral salt is desirable. With such procedure, the crepe of the sheet is not destroyed, nor is it seriously affected, although the solution penetrates the sheet and fixes the dye within the paper fibers, thereby rendering it substantially protected from and relatively insoluble or non-bleeding toward subsequent wetting or other forms of moisture which may come into contact with the sheet. Moreover, if certain inorganic salts are added to or with the fixing reagent, thereby increasing the effective concentration (such as ammonium sulfate in the example cited), the paper is simultaneously rendered slow-burning or fireproof which is an obvious ad-

vantage and secured incidentally to the required operations of dyeing and fixing.

In other cases it may be advantageous, for the purpose of preserving the crepe, as above pointed out, to dissolve the reagent to be applied to the sheet in an organic solvent, which does not soften the paper or cause it to stretch under tension as does water. To this end the reagent (for example, katanol-O which is the reaction product of orthochlorophenol and sulfur in alkaline solution) may be dissolved in alcohol, for example, and the solution thus obtained used to advantage. Again it is contemplated that the fixing reagent may be applied, per se, in an anhydrous condition, as by dissolving in a strictly anhydrous solvent, i. e.  $CCl_4$  or  $C_6H_6$ .

Katanol (By) is a yellowish powder, soluble in hot water with addition of sodium carbonate, and possesses a direct affinity for cotton. 10 parts of sulfur are added to a solution of 26 parts of O-chlorophenol in 20 parts of hot water and 8.5 parts of sodium hydroxide. The mixture is heated immediately to 100° C. under a reflux, and is boiled for 30 hours. The resinous product which separates is dissolved in 200 parts of water and 15 parts of soda, reprecipitated with sodium sulphate, filtered and the greenish paste is dried in vacuo (Fr. Bayer & Co. E. P. 173313; cf. E. P. 22417/95, U. S. P. 603755, G. P. 102897; Guenther, Textilber, 1922, 209; cf. J. S. D. C. 1922, 38,253; Wagner, Farben-Zeit, 1922, 27, 3015).—Color Index, 1924—page 357.

As a modification of the application of the invention, as where the dye solution tends to corrode or accumulate upon the creping rolls, the fixing reagent may be applied to the paper first, followed by creping the paper and applying the dye solution to the treated crepe paper thus produced. This may be effectuated in practice by supplying the solution of fixing reagent to tank 9 and a solution of the dye to tank 16. In this order of operations, an ammoniacal solution of katanol may be used as the fixing reagent in conjunction with a suitable amount of adhesive (and sodium tungstate, if desired, which serves as a fire-proofing agent). The treated sheet is then creped and the dye solution (according to formula three or four given above) may then be applied to the creped sheet already containing the fixing reagent, with or without intermediate drying of the sheet, as required by the conditions of operation.

Accordingly, if the dye solution is applied first, the fixing reagent may be applied later, while if the fixing reagent is applied first, the treatment with the dye solution may be postponed and applied later to the impregnated creped sheet, as desired. In other words, by employing a suitable dye or fixing solution (with substantially no decreping effect) in accordance with the present invention, a creped sheet of paper may be treated

nearly as readily and effectively as the plain sheet before creping and the specific sequence of steps required by other methods (in which the creping is effected last) need not be adhered to. This results in greater flexibility and the ready adaptation of the process to the practical requirements of manufacture and hence facilitates control of the product and of the operation of the method at the several stages of procedure.

The product is characterized by having a uniformity of color and of crepe effect and may be of substantially any predetermined shade or tone desired. The lustre of the surface, which may be enhanced by using a paper having a finished surface on one or both sides is, to an appreciable degree, preserved. This is especially noticeable when an organic solvent is used for the fixing reagent. Again, a fine or coarse degree of creping may be imparted to the sheet as desired, and a high crepe ratio may be obtained and preserved because the subsequent treatment does not seriously impair the crepe finish. Moreover, the finished product is "non-bleeding" and the colors are relatively fast when brought into contact with moisture or even when thoroughly saturated and soaked with water.

It is apparent that numerous modifications and adaptations of the invention may be made in its practical application and that various substitutions and combinations of the raw materials and reagents used may and ordinarily will be required for specific purposes of manufacture and use. Such modifications and substitutions are, however, to be considered as comprehended by the foregoing disclosure and included within the following claims.

This application is a division of application Serial No. 147,959, filed November 12, 1926 issued as Patent 1,756,778, dated April 29, 1930.

I claim:

1. A method for making non-bleeding colored crepe paper, which comprises treating a sheet of paper with a solution of a fixing reagent, creping the treated sheet and thereafter applying a solution of dye to the creped sheet.

2. A method for making non-bleeding colored crepe paper, which comprises treating a sheet of paper with a solution of a fixing reagent and a fireproofing reagent, creping the treated sheet and thereafter applying a solution of dye to the creped paper.

Signed by me at Framingham, Massachusetts, the 31st day of March 1930.

GARDNER R. ALDEN.